

## UNITED STATES PATENT OFFICE.

YOSHICHI SHIBATA, OF NIHONBASHI-KU, TOKYO, JAPAN.

## NAPHTHALENE INSECT TABLET.

No Drawing.

Application filed July 7, 1922. Serial No. 573,434.

*To all whom it may concern:*

Be it known that I, YOSHICHI SHIBATA, subject of the Emperor of Japan, residing at No. 6 Iwatsuki-cho, Nihonbashi-ku, Tokyo, Japan, have invented certain new and useful Improvements in Naphthalene Insect Tablets; and I do hereby declare the following to be a full, clear, and exact description of the invention, such as will enable others skilled in the art to which it appertains to make and use the same.

This invention relates to the method of making naphthalene insect-tablets containing some perfume essence and borneol or camphor. Mix melted naphthalene with perfume and borneol or camphor, and pour the solution obtained by heating at far lower degree than the melting point of the borneol or camphor into water through a funnel provided with a plurality of holes. Tablets are then made from these granules after being congealed in water, by being pressed in a tablet-machine.

Ordinary tablets made by mixing powdered naphthalene with borneol or camphor and a perfuming material, vaporize very unequally. This is probably due to the fact that the perfume vaporizes much more readily than the other materials.

In accordance with the present invention, however, the tablets are found to vaporize very uniformly, giving off constantly a mixture of the vapors of naphthalene, perfuming agent and borneol or camphor in approximately the same proportions, in which they are present in the tablets. This is on account of the very complete and thoroughly intermixing of the ingredients.

The manufacture of these tablets is preferably conducted by melting naphthalene and heating the same to 120° C., some perfume being added, together with 10 to 20% or so of borneol or camphor. The borneol or camphor will be found to readily dissolve in the molten mass. Drops of this are allowed to fall into water, and the sudden cooling converts these drops into granules, which possess a rough exterior and are weak. During this operation the water should be stirred up or should be renewed from time to time to keep the same cold.

The following examples are given of the proportions which may be employed:

*Example 1.*

|                 | Parts. |
|-----------------|--------|
| Naphthalene     | 100    |
| Borneol         | 10     |
| Perfume essence | 5      |

*Example 2.*

|                 | Parts. |
|-----------------|--------|
| Naphthalene     | 100    |
| Camphor         | 15     |
| Perfume essence | 5      |

These materials are, on account of the mode of preparation combined together very thoroughly and hence each material is so held in the tablet that it cannot vaporize independently from the other ingredients, but all of the ingredients together vaporize gradually in about the proportion in which they are mixed in the tablets. The tablets are easily shaped in the tablet-machine from the granules, and it is not necessary to previously grind up the ingredients.

Although the melting point of borneol is 203° C., and that of camphor is 105° C., while the melting point of naphthalene is only 79° C., the affinity of these substances for each other makes a perfect blend on account of the melting and solution of the borneol or camphor in the molten naphthalene.

The expression "a borneol compound" is hereinafter used to embrace both borneol itself and camphor.

I claim:

A method of making naphthalene insect tablets, containing a perfume, which comprises forming a molten mixture of naphthalene, a borneol compound and a perfume, then running this in the form of small masses into cold water to congeal the same, and then pressing the granules into tablet form.

In testimony whereof I affix my signature,

YOSHICHI SHIBATA.

Witness:

N. HARASHIMA.